

## UNITED STATES PATENT OFFICE

2,202,150

## ELECTRIC CONTACTING ELEMENT

Franz R. Hensel and Earl I. Larsen, Indianapolis,  
Ind., assignors to P. R. Mallory & Co., Inc.,  
Indianapolis, Ind., a corporation of Delaware

No Drawing. Application February 24, 1939,  
Serial No. 258,187

2 Claims. (Cl. 219—4)

This invention relates to a new copper base contacting element of improved characteristics.

An object of the invention is to improve the electrical characteristics of the element, such as 5 the electrical conductivity.

Another object is to improve the temperature resistant characteristics of such an element, such as the annealing temperature and the hardness values of the alloy at temperature.

10 Another object of the invention is to improve the hardness and tensile properties of copper base elements of the type disclosed.

Other objects of the invention will be apparent 15 from the following description taken in connection with the appended claims.

The present invention comprises the combination of elements, methods of manufacture and the product thereof, brought out and exemplified in 20 the disclosure hereinafter set forth, the scope of 20 the invention being indicated in the appended claims.

While a preferred embodiment of the invention 25 is described herein, it is contemplated that considerable variation may be made in the method of procedure and the combinations of elements, 25 without departing from the spirit of the invention.

The present invention contemplates a contacting 30 element formed of an alloy of copper, silver and lithium.

The alloy may preferably contain the essential 35 ingredients, in the following proportions:

Silver ..... per cent. .02—15  
35 Lithium ..... do. .002—1  
Copper ..... Balance

Within these compositions ranges, there are a 40 number of specific alloys which have been found to be of particular importance. Several of these 40 alloys are listed below:

- (1) Silver ..... per cent. .03—.08  
Lithium ..... do. .002—.01  
Copper ..... Balance
- 45 (2) Silver ..... per cent. .5  
Lithium ..... do. .002—.01  
Copper ..... Balance
- (3) Silver ..... per cent. 2  
Lithium ..... do. .002—.01  
Copper ..... Balance
- 50 (4) Silver ..... per cent. 6  
Lithium ..... do. .002—.01  
Copper ..... Balance

(5) Silver ..... per cent. 8—12  
Lithium ..... do. .1—.25  
Copper ..... Substantially the balance

In some instances, it may be desirable for cer- 5 tain uses, to effect an improvement in the alloy by adding small percentages of additional in- gredients, such as:

|           |           |    |
|-----------|-----------|----|
| Cadmium   | Zirconium | 10 |
| Zinc      | Thorium   |    |
| Magnesium | Uranium   |    |
| Beryllium | Chromium  |    |
| Calcium   | Cobalt    |    |

Copper-silver alloys have heretofore been used 15 for many purposes, particularly where high elec- trical conductivity was of importance, or where it was necessary to improve the physical properties of pure copper.

One of the outstanding effects of small amounts 20 of silver in copper is that the annealing tempera- ture of such materials is raised considerably. At the same time, silver has a variable solid solubil- 25 ity in copper and therefore, by proper heat treat- ing, or by a proper combination of working and heat treating, almost all of the silver can be made to precipitate from the copper solid solution and therefore, the electrical conductivity can be raised to very high values. While at 779 degrees

C., 8% of silver is held in solid solution, this 30 amount is decreased to 4.5% at 700 degrees; 2.4% at 600 degrees; 1.2% at 500 degrees, .5% at 400 degrees; .25% at 300 degrees, and less than .1% at 200 degrees. The electrical conductivity is de- creased by the formation of solid solutions.

35 Whenever a solid solution is formed, the conduc- tivity will be decreased greatly, due to the spe- cific molecular arrangement of the solid solution 30 crystals. If these solid solutions are decomposed by heat treatment or by a combination of cold

work and heat treatment, then the resulting alloy 40 will consist primarily of two ingredients and the electrical conductivity can be determined by ap- 40 plying a simple rule of mixtures. In cases where

45 the two ingredients have extremely high conduc- tivity, such as copper and silver, then the resulting 45 electrical conductivity will be proportionally very high.

We now have discovered that this precipitation 50 of silver from a copper solid solution, is greatly enhanced by the addition of lithium. The lithium forms a series of alloys and compounds with sil- 50 ver, while it is almost completely insoluble in copper, therefore tending to promote a more com- 55

plete precipitation of the silver phase from the copper matrix.

Our experiments have shown that the addition of lithium in alloys which contain only small percentages of silver, will result in a material which actually has a higher conductivity than pure copper. An alloy, for instance, containing .05% silver, .002% lithium, and the balance copper, will have an electrical conductivity of 101% International Annealed Copper Standard. At the same time, the annealing temperature of such alloys, after severe cold working, is in the neighborhood of 350 to 400 degrees C. If such alloys are used, for instance, for spot welding electrodes, a highly improved performance will result, due to the combination of the extremely high electrical conductivity, the improved Rockwell B hardness, and the increased annealing temperature. Whereas, pure copper will mushroom very rapidly, this new alloy will withstand mushrooming for a much longer time and will allow at least 3 to 5 times the number of welds to be made with a single electrode.

The addition of lithium also eliminates impurities and particularly oxides which may be contained in the melt, and it therefore eliminates the use of such highly detrimental deoxidizers as phosphorus, silicon, etc., which will decrease the electrical conductivity very materially, if present even in small proportions, which are generally classified as impurities.

We do not, however, contemplate the addition of lithium as a deoxidizer only. Sufficient lithium is added to the copper base to insure that the residue thereof, retained in the copper-silver alloy, does not amount to less than the certain desired percentage.

For deoxidizing purposes only, it is also possible to add other elements of the alkali group, or alkaline earth group, or alloys thereof, such as, for instance, sodium or calcium.

The improvements of the alloys of the present invention, characterized by the addition of lithium, are very pronounced also in the case where higher silver contents are used in order to obtain higher strength alloys.

We have found that alloys of this type give excellent performance, if used for electrical contacts and more particularly, contactor contacts. The lithium will tend to keep the surface of the alloy clean, and therefore reduce the contact resistance to a minimum, while the presence of silver improves the hardness and wear resistance of the contacts against mechanical abrasion.

The alloy is exceptionally well adapted to the production of resistance welding electrodes, seam welding wheels and welding dies and fixtures in general.

While the present invention as to its objects and advantages has been described herein, as carried out in specific embodiments thereof, it is not desired to be limited thereby, but it is intended to cover the invention broadly, within the spirit and scope of the appended claims.

What is claimed is:

1. A resistance welding electrode characterized by high electrical conductivity and high hardness, formed of an alloy composed essentially of .002 to 1% lithium, .03 to 8% silver and the balance substantially all copper.

2. An electric contacting element of the type comprising contactor contacts, work-engaging pressure exerting electrodes and the like, said element being characterized by high hardness and high electrical conductivity and formed of an alloy composed essentially of .002 to 1% lithium, .02 to 15% silver and the balance substantially all copper.

FRANZ R. HENSEL.  
EARL I. LARSEN.